

## UNITED STATES PATENT OFFICE

2,138,602

## DYEING OF HARDENED CASEIN

Frederick Hill and Jack Augustus Radley, Blackley, England, assignors to Imperial Chemical Industries Limited, a corporation of Great Britain

No Drawing. Application January 18, 1938, Serial No. 185,624. In Great Britain January 29, 1937

6 Claims. (Cl. 8—4)

The production from casein of hardened masses and articles is well known and such material is manufactured under various trade names. It finds a variety of applications, for instance, in the making of buttons. For the polishing of hardened casein a method employed is to immerse the material in an aqueous hypochlorite solution, e. g. of sodium or calcium hypochlorite, followed by drying. This treatment imparts to the hardened casein a gloss or polish, but renders it difficult to dye.

The dyestuffs used at present are acid dyestuffs. Whereas untreated hardened casein readily takes up acid dyestuffs from an aqueous dye-bath, casein which has been treated with hypochlorite loses much of its affinity for such dyes; only tinctorially weak dyeing can be obtained or it may even be that very little or no colouration of the material can be effected.

A further drawback to the use of ordinary acid dyestuffs for the dyeing of formed casein articles, for instance, buttons, is that uneven dyeings are liable to be produced and their rims or edges are frequently dyed a deeper shade than the remainder.

This invention has as an object to devise a method of dyeing hardened casein which will not have the disadvantage mentioned above. A further object is to provide better dyed casein articles. Further objects will appear hereinafter.

These objects are accomplished by the following invention. We have found that we can dye hardened casein if we employ for the dyeing of this substance monoazo, or anthraquinone dyestuffs containing an oxyalkyl radicle esterified by an acid sulphuric ester group, e. g.



or its salts, attached to an aromatic nucleus by an —O or an —N linkage but which are devoid of sulphonic or carboxylic groups attached directly to an aromatic nucleus.

The following examples illustrate but do not limit the invention. The parts are by weight.

## Example 1

1 part of the dyestuff p-nitraniline→N-ethyl-N-β-hydroxyethylaniline sulphuric ester is dissolved in 5000 parts of water and 200 parts of a 1% formic acid solution added. Buttons made from casein are dyed in this solution for 10 minutes at a temperature of 70° C. and attain a deep and level scarlet colour.

## Example 2

1 part of the dyestuff, p-aminophenyl-β-hydroxyethyl ether sulphuric ester→p-cresol is dissolved in 5000 parts of water and 200 parts of a 1% formic acid solution added. Casein buttons which have been treated with hypochlorite solution are dyed in this solution for 10 minutes at a temperature of 70° C. and acquire a bright and level yellow colour.

## Example 3

1 part of the dyestuff, the sodium salt of the sulphuric ester of 1-methylamino-4-β-hydroxyethylaminoanthraquinone, is dissolved in 5000 parts of water and 200 parts of a 1% formic acid solution added. Thin casein slabs are dyed in this solution for 10 minutes at 70° C. and acquire a deep and level blue colour.

## Example 4

1 part of the dyestuff, the sodium salt of the sulphuric ester of 1-amino-4-β-hydroxyethylamino-2-methylanthraquinone is dissolved in 20,000 parts of water containing 800 parts of a 1% formic acid solution. The temperature of this solution is maintained at 80° C. and casein buttons are immersed in it for 10 minutes, after which they are removed, rinsed in water and dried. The buttons are thus obtained coloured 30 violet.

As many apparently widely different embodiments of this invention may be made without departing from the spirit and scope thereof, it is to be understood that we do not limit ourselves to the specific embodiments thereof, except as defined in the appended claims.

## We claim:

1. A process for the dyeing of hardened casein which comprises applying to the material from a dye-bath a dyestuff of the class consisting of monoazo and anthraquinone dyestuffs which dyestuff contains a hydroxy-alkyl sulphuric ester group attached to an aromatic nucleus through an atom of the class consisting of oxygen and nitrogen and which dyestuff is devoid of any sulphonic and carboxylic groups attached directly to an aromatic nucleus.

2. A process according to claim 1 in which the hardened casein has been polished by treatment with an aqueous hypochlorite solution.

3. A process according to claim 1 in which the hydroxyalkyl sulphuric ester group in the dyestuff is a sulphatoethyl group.

4. A process according to claim 1 in which the

dyestuff employed in the dyebath is an azo dyestuff prepared by diazotizing p-nitraniline and coupling with N-ethyl-N-beta-hydroxyethylaniline sulphuric ester.

5 5. A process according to claim 1 in which the dyestuff employed in the dyebath is an azo dyestuff prepared by diazotizing p-aminophenyl-beta-hydroxyethyl ether sulphuric ester and coupling with p-cresol.

6. A process according to claim 1 in which the dyestuff employed in the dyebath is the sodium salt of the sulphuric ester of 1-methylamino-4-beta-hydroxyethylaminoanthraquinone.

5

FREDERICK HILL  
JACK AUGUSTUS RADLEY.